

May 17, 1927.

1,629,311

W. E. RUDER

MAGNETIC CORE FOR ELECTRICAL MACHINERY

Filed March 12, 1925

Fig.1.



Fig.2.



Inventor:  
William E. Ruder,  
by Alexander S. Lutz,  
His Attorney.

## UNITED STATES PATENT OFFICE.

WILLIAM E. RUDER, OF SCHENECTADY, NEW YORK, ASSIGNOR TO GENERAL ELECTRIC COMPANY, A CORPORATION OF NEW YORK.

## MAGNETIC CORE FOR ELECTRICAL MACHINERY.

Application filed March 12, 1925. Serial No. 15,048.

The present invention relates to the construction of magnetic cores for transformers, dynamo-electric machinery and other electric apparatus.

5 It is the object of my invention to provide a construction whereby the energy losses due to eddy currents in magnetic cores will be reduced, with a consequent increase in the efficiency of operation of the devices 10 of which the cores form a part.

Heretofore the laminations of which the cores of magnetic devices are constituted have been provided with a thin coating of varnish consisting of a gummy or resinous 15 material for the purpose of insulating the laminations from each other. I have found that these materials tend to flow when subjected to the heavy pressures used in assembling large magnetic cores, thus partly 20 destroying their insulating value by bringing the laminations into electrical contact wherever the varnish has been displaced. When the scale which is formed on the laminations during their manufacture is re- 25 moved before coating then the insulating value of a varnish on the sheets is even less effective, and the eddy current losses hence are high.

Ordinary electrical insulation cannot be 30 interposed between the laminations as this would increase the bulk of the core and thus offset any gain in efficiency due to decreased eddy current losses.

I have discovered that the laminations of 35 a core may be effectively insulated by providing the laminations with a thin coating of varnish in which a finely divided solid insulating material has been incorporated, thus producing a film which will not flow 40 under pressure.

The accompanying drawing shows in Fig. 1 a transformer core as illustrative of the class of apparatus to which my invention is applicable; Fig. 2 showing a single sheet or 45 lamination of the core.

In carrying out my invention the sheet material which is to be built up into the cores, for example, silicon steel sheets, such

as shown in Fig. 2, are provided with the desired coating by spraying, painting or by 50 passing through rubber rollers upon which the coating material is applied. Linseed oil, bakelite or other suitable hardening adhesive material into which has been incorporated a substantial proportion, say 20 per cent by 55 weight, of finely divided china clay, silica, mica or other solid insulating material provides a suitable product. The light flaky product obtained by heating phlogopite, a 60 magnesia mica mined at Libby, Montana, makes a desirable filler. Mixtures of different insulating materials sometimes may be used to advantage.

The coated material is baked to set the 65 binder and then is assembled in the usual manner, to form a core such as shown in Fig. 1. The resistance of magnetic cores thus provided with a non-flowing coating is enormously higher than the resistance of a core provided with ordinary varnish. The 70 increase of resistance varies widely from a thousand fold to a hundred thousand fold. The eddy current losses of magnetic cores comprising laminations when coated with a 75 non-flowing material are reduced fifty per cent or even more depending on the nature of the material.

What I claim as new and desire to secure by Letters Patent of the United States, is:—

1. An article of manufacture comprising 80 magnetic sheet material provided with a thin, adherent, electrical insulating, and heat resisting coating, said coating containing varnish and a substantial proportion of finely divided mica.

2. A magnetic core for electrical devices comprising a plurality of laminations of magnetic material, the laminations being provided with thin films of adherent insulating material, said insulating material containing approximately 20 per cent by weight 85 of finely divided mineral insulation, and being capable of withstanding pressure.

In witness whereof, I have hereunto set my hand this 11th day of March, 1925.

WILLIAM E. RUDER.